

(No Model.)

H. A. HOWE.  
Coating for Metallic Chills.

No. 237,281.

Patented Feb. 1, 1881.



Attest:

A. Barthel  
Charles F. Hunt.

Inventor:

Henry A. Howe

By Act

J.W. S. Sprague

# UNITED STATES PATENT OFFICE.

HENRY A. HOWE, OF DETROIT, MICHIGAN.

## COATING FOR METALLIC CHILLS.

SPECIFICATION forming part of Letters Patent No. 237,281, dated February 1, 1881.

Application filed October 23, 1880. (No model.)

*To all whom it may concern:*

Be it known that I, HENRY ARCHIBALD HOWE, of the city of Detroit, in the county of Wayne and State of Michigan, one of the 5 United States of America, gentleman, have invented certain new and useful Improvements in a Coating for Metallic Chills; and I do declare that the following is a full, clear, and exact description of the same.

10 My invention relates to improvements in coating metallic chills, whereby a casting provided with holes having parallel sides may be formed by means of a chill having parallel sides; and to this end the improved coating 15 to be applied to the outer surface of the chill consists of petroleum or oleaginous matter covered by plumbago, as hereinafter more fully set forth.

The greatest utility of coating will be found 20 in casting pulleys, wheels, and other similar articles, such as are compelled to be bored out true to fit upon or run on shafts or axles, for by the application of this coating to the outer surface of a chill with parallel sides a perfectly true hole, perfectly straight, and with parallel sides, and smooth enough to run upon a shaft or axle, can readily and easily be obtained, thereby avoiding the expense and trouble of boring, while at the same time all 25 the benefits derived from a chilled surface will be had.

The figure is a vertical central section through a wheel molded in the sand, with the core-chill in place, resting in the sand-core 30 prints.

In the accompanying drawing, which forms a part of this specification, A represents a round, straight steel shaft or core-chill, with parallel sides of that portion of it from a to b, 35 which is designed for chilling purposes. This portion of the chill is prepared for use by thinly and evenly being coated with petroleum or oleaginous matter, to which is applied thinly and evenly a coating of plumbago which has

been pulverized to an almost impalpable powder. 45

The wheel B is molded in the ordinary manner, and after the pattern is removed from the sand the core-chill is placed in the sand-core prints. If it is desired that the ends of the 50 hub of the wheel be even and true, the core-chill may be provided with flanges c, one of which may be rigidly secured to the chill, and the other may be in the form of a ring to slip onto the chill for convenience in adjusting it, 55 or both flanges may be removable.

After the casting is poured in the usual way, in cooling the iron shrinks, and were it not for the coatings on the core-chill the iron would so closely embrace it that it could not be withdrawn, nor could the shaft or chill be rotated; but the heat of the iron slowly decomposes the 60 petroleum, which is prevented from burning by the intervening coating of plumbago, which latter leaves a smooth surface on the chilled 65 iron, the two coatings forming a cushion to prevent the cooling iron from so thoroughly embracing the core-chill that it may not be easily and readily removed.

It will be observed that a coat or layer of 70 the petroleum is first applied to the chill, and that a layer or coat of plumbago is afterward applied to the chill over the petroleum, which I prefer to a compound of the petroleum and plumbago.

75 What I claim as my invention is—

1. A coating for metallic chills, consisting of petroleum or oleaginous matter covered with a layer of plumbago, as and for the purpose set forth. 80

2. A chill with parallel sides coated with petroleum or oleaginous matter and a superposed layer of plumbago, substantially as described, and for the purpose set forth.

HENRY A. HOWE.

Witnesses:

CHARLES J. HUNT,  
H. S. SPRAGUE.